

## UNITED STATES PATENT OFFICE.

STUART CROASDALE, OF DENVER, COLORADO.

## PROCESS FOR THE CONCENTRATION OF OXIDIZED ORES.

No Drawing.

Application filed January 8, 1923. Serial No. 611,473.

*To all whom it may concern:*

Be it known that I, STUART CROASDALE, a citizen of the United States, residing at Denver, in the county of Denver and State of Colorado, have invented certain new and useful Improvements in Processes for the Concentration of Oxidized Ores, or which the following is a specification.

My invention relates to a process of concentrating ores by flotation and its primary object resides in subjecting comminuted ores in the process of concentration commonly known in the art as a flotation process, to a novel treatment whereby those of their mineral particles which heretofore have not been amenable to concentration, are made subject to the affinity and the buoyant influence of a flotation agent.

The present application is a continuation in part of my application for patent Serial No. 503,355, filed September 26, 1921.

My invention is particularly adapted for the treatment of oxidized ores, it being a well known metallurgical fact that minerals of oxidized character do not adsorb the oleic or gaseous re-agents to an extent necessary for their flotation, and, therefore, cannot be concentrated as readily by a flotation process as those consisting entirely or in part of sulfides.

My process consists briefly in mixing the ore under treatment in a finely divided state, with a soluble sulfide re-agent, a frothing agent and an oil or other hydrocarbon compound containing a substantial percentage of what are generally termed unsaturated hydrocarbons such as are contained in mineral oils, either in their natural condition or artificially obtained.

The unsaturated hydrocarbons suitable for use in the process are more particularly those which belong to the olefine series.

The action of the sulfide re-agent upon the oxidized ore particles causes a physical change in their surface character which renders them capable of ready flotation in the usual manner by oils or hydrocarbons of the kind hereinabove referred to, with the addition of a suitable frothing agent, as for example, pine oils or wood or coal tar creosotes and other products of their distillation.

It is desired to clearly indicate that in order to effect a successful flotation and re-

covery of the oxidized constituents, the unsaturated hydrocarbon must be added in addition to the frothing agent. Some of the commonly used frothing agents, including those mentioned, may contain a small percentage of unsaturated hydrocarbons but the presence of the same in the amount usually used for flotation, namely, one-half to one pound per ton of ore, is relatively negligible and it is only when a considerable quantity of the unsaturated hydrocarbons, preferably of the olefine series are present, that a successful recovery of the oxidized ore occurs.

Examples of the unsaturated hydrocarbons which I prefer to use are as follows:

1. A crude petroleum of paraffin or asphaltic base but preferably the former, containing the highest obtainable percentage of unsaturated hydrocarbons. Crude petroleums contain, as a rule, from 15% to 90% unsaturated hydrocarbons.

2. Distillation fractions of crude petroleum having the approximate viscosity of the gas oil fraction and containing their relative percentages of unsaturated hydrocarbons. In stating "the approximate viscosity of the gas oil fraction", I include with the gas oil fraction the kerosene fraction on one side and the light lubricating oil fraction on the other.

3. Products obtained from "cracking" petroleum under pressure, which have still higher percentages of unsaturated hydrocarbons than the original crude petroleum.

4. Unrefined products obtained from the distillation of oil shales, which contain from 30% to 80% of unsaturated hydrocarbons, according to the method of distillation. These oils contain a high percentage of unsaturated hydrocarbons due to the partial "cracking" of the oils during distillation.

The change produced on the surface of the mineral particles consists in their envelopment by a thin adsorbed coating or film of the sulfide re-agent produced by the chemical affinity of the sulfide re-agent for the mineral without chemical re-action noticeable to the naked eye.

While there is a possibility of a slight chemical reaction taking place on the surface of the oxidized minerals in order to cause them to adsorb the films of the re-

agent, the use of oils or hydrocarbon compounds of the above mentioned character containing a substantial percentage of unsaturated hydrocarbons eliminates the necessity of sulfidization required by other oils or hydrocarbons commonly used in a flotation process.

In carrying out my invention, the ore is ground in any suitable manner to a fineness sufficient to liberate the mineral from the gangue and is mixed together with the hydrocarbonaceous compound, the sulfide re-agent and a frothing agent, in water to form a pulp of the consistency usually used in the flotation process.

In this connection, it will be understood that the oil, the sulfide re-agent and the frothing agent may be added while the material is being ground instead of afterward should this method of intermixing the ore and ingredients be found to be more convenient or efficient in handling a particular grade or kind of crude material.

The ore pulp is fed into a tank of the kind usually employed in a flotation process and the hydrocarbon compound acting upon the oxides coated by the sulfide re-agent, causes with the addition of a frothing agent, a concentration of these minerals at the surface of the liquid mass from where they are removed in an overflowing froth as usual.

The quantities in which the sulfide re-agent, the hydrocarbon compound and the frothing agent are used must necessarily be varied in accordance with the nature of the material under treatment, it being evident that by reason of the infinite variations in the composition of ores, no definite proportions can be relied upon for the successful application of the present process to different ores and under different conditions.

As an example, in the treatment of a copper ore having a total copper content of 3.4% of which 1.78% was sulfides of copper and 1.62% oxidized copper, it was found advantageous to use to each ton of the material 20 pounds of an approximately 30% solution of calcium poly-sulfide, 4 pounds of mineral oil (crude petroleum containing 68% of unsaturated hydrocarbons), and from  $\frac{1}{4}$  to  $\frac{1}{2}$  pound of a frothing agent (hard wood creosote). In treating the mixture by the flotation process, 85% of the oxidized copper was concentrated at the surface of the liquid, after a commercial recovery of the sulfides of copper had been made in the usual manner.

In a treatment of a lead silver ore containing 6.7 ounces of silver per ton and 7.3% of lead in an oxidized condition, were used to each ton of the material 20 pounds of the above mentioned solution of calcium poly-sulfide, 4 pounds of shale oil containing approximately 60% of unsaturated hydrocarbons, and a frothing agent consisting of

from  $\frac{1}{2}$  to one pound of hard wood creosote. The result was the recovery of 94% of the silver and 96.9% of the lead.

The sulfide re-agents best adapted for use in my process of concentration are the poly-sulfides of the alkaline earth metals and more particularly the poly-sulfides of calcium. By the use of these poly-sulfides, the efficiency of the process is not impaired by the introduction of soluble salts since only salts of a very low degree of solubility are entered into the material.

The use of poly-sulfides of the alkaline earth metals furthermore is advantageous in that they insure the presence of a higher percentage of active sulfur in combination with the alkaline earth metal than is obtainable in the use of the normal monosulfides or di-sulfides of the same metals, it being observed that the highest filming actions are obtained with a minimum alkalinity of the ore pulp.

Still another advantage of the use of poly-sulfides of the alkaline earth metals and more particularly the poly-sulfides of calcium, resides in the simple manner in which this compound may be prepared and the low cost at which it can be produced.

Among the various poly-sulfides of the alkaline earth metals, penta-sulfide of calcium has been found to be particularly suitable as a re-agent in my improved flotation process.

Under certain conditions, the sulfides of the alkaline metals or hydrogen sulfides may be found to give satisfactory results although the poly-sulfides of the alkaline earth metals are more desirable since alkaline metal sulfides have a strong sulfidizing action which is undesirable in the present process, and since their presence distinctly interferes with the formation of a froth in which the minerals are collected.

Alkaline metal sulfides furthermore produce an excess of alkalinity in the ore pulp and thereby prevent efficient commercial recovery of the values.

I am aware that the use of sulfide re-agents in a flotation process has been heretofore attempted and I desire it understood that my invention resides not in the use of a sulfide re-agent as a means for sulfidization, but in its use for the production of an adsorbed coating of the sulfide re-agent upon the oxidized mineral particles by which the commercial recovery of said particles in their natural state by use of an oil or other hydrocarbon containing unsaturated hydrocarbons, in conjunction with a suitable frothing agent, is made possible.

It should be understood that my improved process resides particularly in the production of an adsorbed film on the surface of the oxidized mineral particles and that no change takes place in the ore pulp.

mixture as in other processes heretofore used for the same purpose, and it should also be noted that in my process there is no visible chemical re-action between the sulfide re-agent and the oxidized mineral particles.

It will furthermore be evident that the process is also beneficial in the treatment of partially oxidized ores where the residual sulfide particles of mineral may be coated 10 with an oxidized surface.

The terms "hydrocarbons containing a substantial percentage of unsaturated hydrocarbons" and "hydrocarbons containing a substantial percentage of unsaturated hydrocarbons of the olefine series" as used in 15 the claims is to be interpreted to mean those compounds which outside of minor impurities are substantially composed of hydrogen and carbon. It specifically excludes the hydrocarbon derivatives such as the oxygen 20 compounds known under the name of alcohols or sulphonated hydrocarbon compounds.

Having thus described my invention, 25 what I claim and desire to secure by Letters Patent is:

1. The process of concentrating by flotation ores containing oxidized minerals to more completely recover the same, the flotation being accomplished without forming 30 any visible film of metallic sulfide on the surfaces of the mineral particles, comprising treating the ore-pulp in the presence of calcium pentasulfide, a frothing agent, a 35 relatively large amount of a hydrocarbon containing a substantial percentage of unsaturated hydrocarbons of the olefine series and recovering the concentrates.

2. The process of concentrating by flotation ores containing oxidized minerals to more completely recover the same, the flotation being accomplished without forming any 40 visible film of metallic sulfide on the surface of the mineral particles, comprising

treating the ore-pulp in the presence of 45 calcium polysulfide, a frothing agent and a relatively large amount of a hydrocarbon containing more than 50% of unsaturated hydrocarbons of the olefine series and recovering the concentrates.

3. The process of concentrating by flotation ores containing oxidized minerals to more completely recover the same, the flotation being accomplished without forming 50 any visible film of metallic sulfide on the 55 surfaces of the mineral particles, comprising treating the ore-pulp in the presence of calcium pentasulfide, a frothing agent, a relatively large amount of a hydrocarbon containing a substantial percentage of unsaturated hydrocarbons and recovering the 60 concentrates.

4. The process of concentrating by flotation ores containing oxidized minerals to more completely recover the same, the flotation being accomplished without forming 65 any visible film of metallic sulfide on the surfaces of the mineral particles, comprising treating the ore-pulp in the presence of calcium polysulfide, a frothing agent, a 70 relatively large amount of a hydrocarbon containing a substantial percentage of unsaturated hydrocarbons and recovering the 75 concentrates.

5. The process of concentrating by flotation ores containing oxidized minerals to more completely recover the same, the flotation being accomplished without forming any visible film of metallic sulfide on the 80 surfaces of the mineral particles, comprising treating the ore-pulp in the presence of a polysulfide, a frothing agent, a relatively 85 large amount of a hydrocarbon containing a substantial percentage of unsaturated hydrocarbons and recovering the concentrates.

In testimony whereof I have affixed my signature.

STUART CROASDALE.